

Dec. 25, 1945.

A. B. RICHARDS ET AL

2,391,516

PURIFICATION OF LOW MELTING POINT ALLOYS

Filed June 16, 1943



A. B. Richards  
J. T. O'Reilly  
INVENTOR.

BY *Edwin C. Nichols*  
*D. G. Farris*  
*J. Horneys.*

## UNITED STATES PATENT OFFICE

2,391,516

PURIFICATION OF LOW MELTING  
POINT ALLOYS

Alvin B. Richards and James T. O'Reilly, Dearborn, Mich., assignors to Ford Motor Company, Dearborn, Mich., a corporation of Delaware

Application June 16, 1943, Serial No. 490,978

2 Claims. (Cl. 266—34)

This invention relates to the salvage treatment of low melting point metal alloys and, more particularly, to a method of purification of such alloys for re-use in tube-bending operation.

The principal advantage of this invention is that it furnishes a means by which low melting point alloys of the general Woods' metal type, which are commercially known as "Cerro-bend" and under other proprietary names or trademarks, may be salvaged, purified, and made available for continuous re-use in tube-bending operations. In this work, tubes of aluminum or other metals used in aircraft construction, are filled with fluid metal which, because of its low melting point, does not adversely affect the tube structure itself. The alloy is allowed to solidify in place and then the composite tube and its alloy filling are bent by automatic bending machines or other means to the precise alignment and configuration required. The use of the alloy filler, of course, permits the bending operation to be carried out without buckling or extreme deformation of the pipe from the desired circular cross section. After the conformation is obtained, the alloy filling is melted out by placing the tube in hot water, which filling may be salvaged for re-use. While the term "Woods' metal" is used herein, it will be understood that equivalent alloys having substantially a bismuth, tin, lead and cadmium content and characterized by a low melting point are comprehended within its terms.

However, successive re-use of the alloy builds up its impurity content and in time it becomes so contaminated with oxide, slag, debris, etc., as to be unusable for the purpose described. These impurities, investigation has shown, include:

1. Salts deposited by the water which evaporates in the filling and melting-out tanks.
2. Oxides and hydroxides of the metals making up the alloys.
3. Small amounts of dissolved aluminum.
4. Dirt introduced by allowing the metal to spill on the floor during some stage of the process.

While these included impurities have considerable effect upon the characteristics of the alloy in use, they actually constitute a very small percentage of the total volume of the metal. As Woods' metal with its composition of:

Per cent

|         |     |
|---------|-----|
| Bismuth | 50  |
| Lead    | 25  |
| Cadmium | 12½ |
| Tin     | 12½ |

is rather heavy, having a specific gravity of about 10.7, and the specific gravity of the various oxides

and hydroxide formed varies from 5.6 to 9.0, it is apparent that these lighter impurities as well as most of the salts and the dirt described in the Classes 1, 2 and 4 above may be removed by gravity separation. However, the heavier hydroxides and the dissolved materials require chemical treatment for removal. While means of attacking this problem are available to laboratory or research chemists, the purpose of the present invention is to devise a method which is substantially automatic and requires no particular skill or maintenance in its operation, yet which will yield a continuous supply of purified Woods' metal for re-use in the tube-bending process.

The practical advantage is at once apparent when it is considered that the alloy sells at approximately \$.75 per pound and, particularly at the present, incorporates strategic materials such as tin and cadmium which must be conserved at all costs. At the same time, a typical pipe bending installation may produce upwardly of 10,000 pounds of the contaminated metal per month. Heretofore, this metal has been unavailable for further use and represented a substantial loss unless it were subjected to a precisely controlled reconstituting technique. The apparatus disclosed and the method of its operation permit the economical salvage of the metal without deterioration in quality or diminution in quantity and by means which are safe in operation, economical in structure, and practically automatic in operation.

With these and other objects in view, the invention consists in the arrangement, construction and combination of the various parts of the improved device, described in the specification, claimed in the claims, and illustrated in the accompanying drawing in which:

40 Figure 1 is a vertical transverse sectional view through a purification plane setup.

Referring to the drawing, a gravity separating device is indicated generally at 10, an acid-treating tank at 11, neutralizing bath at 12 and pigging molds at 13. The gravity separator includes a tank 14 to which molten impure Woods' metal is supplied through the pipe 15, controlled by the valve 16. This tank, as is each of the others, is provided with a water jacket 17 to maintain the temperature of the alloy above 180 degrees Fahrenheit, so that it will remain molten at all stages in the operation. After introduction of the molten impure alloy to the tank 14, the lighter components, as described heretofore, separate in the form of a slag 18 which may be drawn off at

intervals through the pipe 19 controlled by the valve 20 and this step, in general, may take from one to two hours, the slag tapping preventing further oxidation of the metal. A suitable depth gauge 21 is provided to show the amount of material present in the tank 14. The heavier alloy 22 in the tank 14 is drawn off through the pipe 23, regulated by the valve 24 to flow therefrom in small droplets 25. These flow down the trough 26 into the rubber-lined tank 27 which is again water jacketed at 28 and heated by steampipes 29. This tank contains a hydrochloric acid solution which, for best results, should be maintained at about 20 per cent hydrochloric acid by volume or 8 per cent by weight.

Since the alloy is in the form of small droplets and is intimately mixed in transit through the bath 30 by passing over baffles 31, the heavier oxides, etc., and the dissolved materials are subjected to the hydrochloric acid which precipitates them in the form of a sludge which eventually builds up on the bottom of the tank. However, as the amount of these impurities is relatively small, the sludge forms very slowly and it is only necessary to remove it at infrequent intervals. The alloy continues on its course as shown and finally collects in a sump 32 from which it is withdrawn by the pipe 33 controlled by the valve 34 and again discharged in the form of droplets 35, the trough 36 leading to the neutralizing bath 12.

The neutralizing bath 12 again includes a water-jacketed tank 37 containing a weak sodium bicarbonate or equivalent alkaline solution which washes and neutralizes the metal droplets entering it. These build up into a considerable amount of purified alloy 38 at the bottom of the tank which may be withdrawn through the pipe 39 controlled by the valve 40 and poured into the pigging mold 13 for solidification into individual cakes.

It will be noted that the apparatus devised in this operation is extremely compact and may be operated without technical control. Indeed, it will be found that it may be operated substantially in a continuous manner, the only attention required being periodic replenishment of impure alloy and the drawing off of the pure alloy and its casting in the pig mold. These factors are important because of the immense volume of the metal used in typical pipe-bending installation and the fact that its ready and economic purification permits its reconstitution at frequent intervals with consequent improvement in the characteristic of the metal in actual use. Heretofore, because of the expense involved, it was

necessary to use the metal to its practical exhaustion point which meant that as it was reused, its affecting metal point varied and its homogeneity decreased. Using the present apparatus, it is perfectly feasible to purify the metal at frequent intervals with consequent improvement in its working quality.

Some changes may be made in the arrangement, construction and combination of the various parts of the improved device without departing from the spirit of the invention, and it is the intention to cover by the claims such changes as may be reasonably included within the scope thereof.

15. The invention claimed is:

1. In an apparatus for the purification of used Woods' metal and similar low melting point alloys, a settling tank to hold impure molten alloy, means to maintain the temperature of said tank above the melting point of said alloy, means on said tank to remove the lighter separable portion of the charge therefrom, means to discharge the heavier remainder of said alloy from said tank in the form of minute droplets and to direct said droplets into a second tank containing an acidic solution, means to maintain the temperature of said second tank above the melting point of said alloy, means on said second tank to discharge the accumulated alloy therefrom in the form of minute droplets to a third tank containing a neutralizing bath, means to maintain the temperature of said neutralizing bath above the melting point of said metal, and means to withdraw the metal from said neutralizing bath.
2. In an apparatus for the purification of used Woods' metal and similar low melting point alloys, a settling tank designed to receive said impure molten alloy, means to maintain the temperature within said tank above the melting point of said alloy, means to withdraw the lighter portion of said charge from said tank, gravity means in communication with said tank to discharge the heavier portion of the charge therefrom in the form of minute droplets and to convey said droplets to a second tank containing an acidic bath, means to maintain the temperature of said acidic bath above the melting point of said alloy, gravity means to discharge the accumulated alloy from said second tank in the form of minute droplets and to convey it to a third tank containing a neutralizing bath, means to maintain the temperature in said third tank above the melting point of said alloy, and means to withdraw said metal from said third tank.

ALVIN B. RICHARDS.  
JAMES T. O'REILLY.